



US006110629A

# United States Patent [19]

Ehara et al.

[11] Patent Number: 6,110,629

[45] Date of Patent: \*Aug. 29, 2000

[54] ELECTROPHOTOGRAPHIC,  
PHOTOSENSITIVE MEMBER AND IMAGE  
FORMING APPARATUS

[75] Inventors: **Toshiyuki Ehara; Yuji Nakayama**,  
both of Yokohama; **Tetsuya Karaki**,  
Shizuoka-ken; **Hironori Owaki**,  
Mishima, all of Japan

[73] Assignee: **Canon Kabushiki Kaisha**, Tokyo,  
Japan

[\*] Notice: This patent issued on a continued pros-  
ecution application filed under 37 CFR  
1.53(d), and is subject to the twenty year  
patent term provisions of 35 U.S.C.  
154(a)(2).

[21] Appl. No.: 09/310,987

[22] Filed: May 13, 1999

[30] Foreign Application Priority Data

May 14, 1998 [JP] Japan ..... 10-132245  
May 15, 1998 [JP] Japan ..... 10-133896

[51] Int. Cl.<sup>7</sup> ..... G03G 5/10; G03G 5/082;  
G03G 15/00

[52] U.S. Cl. ..... 430/84; 430/69; 430/95;  
399/159

[58] Field of Search ..... 430/69, 84, 95

[56] References Cited

U.S. PATENT DOCUMENTS

4,461,820 7/1984 Shirai ..... 430/65  
4,689,283 8/1987 Fumiuki et al. ..... 430/69

|           |        |                      |         |
|-----------|--------|----------------------|---------|
| 4,689,284 | 8/1987 | Kawamura et al. .... | 430/84  |
| 4,814,248 | 3/1989 | Kamata et al. ....   | 430/69  |
| 4,895,784 | 1/1990 | Shirai ....          | 430/69  |
| 5,191,381 | 3/1993 | Yuan ....            | 399/90  |
| 5,592,274 | 1/1997 | Higashi et al. ....  | 399/174 |
| 5,595,848 | 1/1997 | Ohtaka et al. ....   | 430/69  |
| 5,729,800 | 3/1998 | Ohba et al. ....     | 399/159 |
| 5,923,925 | 7/1999 | Nakumura et al. .... | 399/159 |
| 5,943,531 | 8/1999 | Talai et al. ....    | 399/159 |

FOREIGN PATENT DOCUMENTS

|           |         |           |
|-----------|---------|-----------|
| 2746967   | 4/1979  | Germany . |
| 2855718   | 6/1979  | Germany . |
| 53-146341 | 12/1978 | Japan .   |
| 55-40161  | 10/1980 | Japan .   |
| 59-191065 | 10/1984 | Japan .   |
| 63-91664  | 4/1988  | Japan .   |
| 63-121851 | 5/1988  | Japan .   |
| 63-210864 | 9/1988  | Japan .   |
| 01-238677 | 9/1989  | Japan .   |
| 02-251866 | 10/1990 | Japan .   |
| 62-175781 | 8/1997  | Japan .   |

Primary Examiner—Roland Martin  
Attorney, Agent, or Firm—Fitzpatrick, Cella, Harper & Scinto

[57] ABSTRACT

A cylindrical, photosensitive member is disclosed which has a photosensitive layer comprising amorphous silicon provided on an electroconductive substrate, and in which the thickness of the electroconductive substrate is not less than 0.1 mm but less than 2.5 mm, thereby accomplishing cost reduction of the photosensitive member and also accomplishing prevention of variations of image density and image smearing by high-accuracy temperature control.

8 Claims, 9 Drawing Sheets



***FIG. 1A******FIG. 1B***

FIG. 2



FIG. 3



FIG. 4



*FIG. 5A**FIG. 5B*

***FIG. 6******FIG. 7******FIG. 8A******FIG. 8B***

FIG. 9



FIG. 10



***FIG. 11******FIG. 12***

FIG. 13



## 1

**ELECTROPHOTOGRAPHIC,  
PHOTOSENSITIVE MEMBER AND IMAGE  
FORMING APPARATUS**

**BACKGROUND OF THE INVENTION**

1. Field of the Invention

The present invention relates to an electrophotographic, photosensitive member and an image forming apparatus having the photosensitive member and, more particularly, to an electrophotographic, photosensitive member capable of achieving lower cost and an image forming apparatus (electrophotographic apparatus) making use of the so-called electrophotographic system having the photosensitive member.

2. Related Background Art

It is required that a photoconductive material for forming a photoconductive layer in an image forming member for electrophotography in the field of formation of image have the following characteristics; for example, having high sensitivity, a high S/N ratio [photocurrent (Ip)/dark current (Id)], absorption spectral characteristics matched with spectral characteristics of an electromagnetic wave radiated thereto (which is light in a general sense, such as ultraviolet light, visible light, infrared light, X-ray,  $\gamma$ -ray, or the like), quick optical response, and a desired dark resistance, being nonpolluting to human bodies during use, and so on. Particularly, in the case of the image forming members for electrophotography incorporated in electrophotographic apparatus used as business machines in offices, the above-stated nonpolluting property during use is a significant point.

On the basis of this viewpoint, for example, German Patent Application Laid-Open Nos. 2746967 and 2855718 describe the application of amorphous silicon in which dangling bonds are compensated with a univalent element such as hydrogen (H), halogen (X), or the like (hereinafter referred to as a-Si(H,X)), to the image forming members for electrophotography, and such materials are applied to the image forming members for electrophotography because of their excellent photoconductive property, wear resistance, and heat resistance, and relative easiness of increase of area to a larger area.

In producing a photosensitive drum for electrophotography having the photoconductive material containing a-Si(H, X), in order to obtain good photoconductive characteristics, it is common practice to deposit an a-Si(H,X) film in the thickness of 1 to 100  $\mu\text{m}$  on a drum-like metal substrate under such a condition that the drum-like metal substrate is continuously heated at relatively higher temperature, 200° C. to 350° C., than in the case of Se-based materials, in an a-Si(H,X) film deposition system. This maintenance of heating of the substrate at the high temperature is necessary for production of the a-Si-based photosensitive drum with excellent electrophotographic characteristics and it is the present status that this maintenance of heating at the high temperature ranges from several hours to somewhat more than 10 hours, based on consideration of deposition rates of the a-Si(H,X) film.

The photoconductive member for electrophotography, in its preferred embodiment, is constructed in such structure that a drum-like, or cylindrical, metal substrate of Al or an Al alloy or the like (hereinafter referred to as an Al-based substrate) is used as a metal support for the photoconductive member for electrophotography and that a photoconductive layer containing an amorphous material having the matrix of silicon and preferably containing at least either one of hydrogen and halogen as a constituent element is formed on

## 2

the drum-like Al-based metal substrate. The photoconductive layer may have a blocking layer in contact with the drum-like metal substrate and further have a surface blocking layer in the surface of the photoconductive layer.

5 FIGS. 1A and 1B are views for explaining an example of the layer structure of the a-Si photosensitive member.

FIG. 1A is a schematic, perspective view, in which reference numeral 2100 indicates the thickness of the photosensitive member including a support 2101 and a photo-receptive layer 2105.

10 FIG. 1B is a schematic, sectional view, in which on the electroconductive substrate 2101 of aluminum or the like there are successively stacked layers, i.e., a charge injection inhibiting layer 2102 for inhibiting injection of charge from the conductive support 2101, and a photoconductive layer 2103 for creating electrons and holes with irradiation of light and converting image information to potential information. Each of these layers is comprised of a material having the matrix of amorphous silicon and, if necessary, containing a neutralizer of the dangling bonds, such as hydrogen and/or halogen, or the like, a valency controller of an element belonging to Group III, Group V, or the like, a modifying substance such as oxygen, carbon, nitrogen, or the like, and so on as occasion may demand. On the upper surface of the photoconductive layer 2103 in the figure, there is provided a surface protecting layer 2104 for protecting the photoconductive layer from friction or the like against a developer, a transfer sheet, a cleaning device, etc. and for preventing charge from being injected from the surface to the photoconductive layer. The surface protecting layer 2104 is comprised of a material of a-SiC:H with excellent light transmittancy to the photoconductive layer, excellent mechanical strength, excellent effect of preventing injection of charge from the top, and so on.

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 987

charge receptibility or the like and the blocking layer is constructed in a single layer or in multiple layers of a-Si(H, X) or polycrystal-Si containing III atoms, V atoms, oxygen atoms, carbon atoms, germanium atoms, etc. according to the purpose.

The layer above the photoconductive layer may be provided as a surface charge injection inhibiting layer or as a protecting layer, which is a layer comprised of an amorphous material having the matrix of silicon atoms, containing carbon atoms, nitrogen atoms, oxygen atoms, etc., preferably, in a large amount and, if necessary, containing hydrogen atoms or halogen atoms, or a layer comprised of a high-resistance organic substance.

The photoconductive layer comprised of a-Si(H,X) is formed by conventionally known vacuum deposition methods utilizing various discharge phenomena, for example, such as a glow discharge method, a sputtering method, an ion plating method, and so on.

Next described is an example of a method for producing the photoconductive member (photosensitive member) for electrophotography by the glow discharge decomposition method.

FIG. 2 shows an example of a system for producing the photosensitive member for electrophotography by the glow discharge decomposition method. A deposition chamber 1 is constructed of a base plate 2, a wall 3, and a top plate 4, and a cathode electrode 5 of a cylindrical shape is provided inside the deposition chamber 1. A drum-like metal substrate 6 on which an a-Si(H,X) deposited film is to be deposited is set in the central part of the cathode electrode 5 (at the center of concentric circles) and also serves as an anode electrode.

For forming the a-Si(H,X) deposited film on the drum-like metal substrate by this production system, first, a source gas inflow valve 7 and a leak valve 8 are closed and an exhaust valve 9 is opened to evacuate the inside of the deposition chamber 1. When the reading of a vacuum gage 10 reaches about  $5 \times 10^{-6}$  Torr, the source gas inflow valve 7 is opened to allow a source mixture gas, for example, of SiH<sub>4</sub> gas, Si<sub>2</sub>H<sub>6</sub> gas, SiF<sub>4</sub> gas, etc., adjusted at a predetermined mixture ratio in a mass flow controller 11 to flow into the deposition chamber 1. At this time the ratio of the value opening of the exhaust valve 9 is adjusted by checking the reading of the vacuum gage 10 so that the pressure inside the deposition chamber 1 becomes a desired value. After it is confirmed that the surface temperature of the drum-like metal substrate 6 is set at a prescribed temperature by a heater 12, a high-frequency power supply 13 is set to a desired power to bring about glow discharge in the deposition chamber 1.

During execution of formation of the layer the drum-like metal substrate 6 is rotated at a constant rate by a motor 14 in order to uniformly deposit the layer. The a-Si(H,X) deposited film can be formed on the drum-like metal substrate 6 in this way.

However, because of the difference between coefficients of thermal expansion of the drum-like metal substrate and the a-Si(H,X) film and large internal stress in the a-Si(H,X) film formed, it was not rare to encounter peeling of the a-Si(H,X) film off the drum-like metal substrate, not only during the deposition of the a-Si(H,X) film in which the drum-like metal substrate was maintained as heated at the high temperature, as described previously, but also during the period of cooling down to the temperature of the outside atmosphere after the deposition. Further, there were more than a few cases in which the a-Si(H,X) film was peeled off because of heating of the drum depending upon the tem-

perature of the operating environment during the use as a photosensitive drum for electrophotography. The film peeling off in the case of the a-Si(H,X) film occurred more readily as the thickness of the a-Si(H,X) film became larger.

With thermal deformation of the drum-like metal substrate (which is, particularly, easy to occur during the formation of the photoconductive layer) even in such a degree as not to cause the film to peel off in the case of the conventional Se-based electrophotographic, photosensitive drums, there were more than a few cases in which the film peeling off occurred in the case of the a-Si(H,X)-based photosensitive drums, for the reason of the aforementioned difference between coefficients of thermal expansion and the magnitude of the internal stress in the a-Si(H,X) film. The internal stress in the a-Si(H,X) film can be relaxed to some extent by production conditions of the a-Si(H,X) film (kinds of source gases, a ratio of flow rates of the gases, discharge power, the heating temperature of the substrate, the internal structure of the production system, etc.), but production conditions are not yet sufficient yet when consideration is given to productivity and mass productivity. This film peeling off will cause image defects and be fatal in application to the photosensitive drum for electrophotography.

The high-temperature heating of the drum-like metal substrate over a long period during the production of the a-Si(H,X) film can be the cause of the above film peeling off and also make the thermal deformation of the drum-like metal substrate happen more readily. This thermal deformation causes nonuniformity of discharge during the production of the a-Si(H,X) deposited film, whereby evenness of thickness of the a-Si(H,X) deposited film is lost, which would be the cause of the image defects.

In view of the various points discussed above, an example of the photoconductive member for electrophotography intended to reduce the image defects is one in which the drum-like metal substrate is comprised of aluminum or an aluminum-based alloy and the thickness is not less than 2.5 mm, for example, as described in Japanese Patent Publication No. 6-14189.

Taking the recent cutthroat price competition and, particularly, development to middle- and low-speed models into consideration making operating cost low is not enough, and the point is how much the initial cost can be decreased. Therefore, an urgent necessity was to decrease the cost of the photoconductive member drastically.

The percentage of the raw material cost was large in the cost of the photoconductive member and decrease in the thickness of the drum-like metal substrate was thus expected to realize not only simple reduction of the raw material cost, but also additional cost reduction, including power savings and decrease in tack time resulting from decrease of the heating time during the production of the a-Si(H,X) film, a cutback of the power for maintaining the high temperature, decrease in the tack time resulting from reduction of the cooling time, and so on, for the reason of the low heat capacity resulting from the small thickness. Therefore, there were urgent desires for cost reduction of the drum-like metal substrate and improvement in temperature characteristics.

#### SUMMARY OF THE INVENTION

The present invention has been accomplished in view of the above problems and an object of the present invention is to provide an electrophotographic, photosensitive member and an image forming apparatus capable of stably providing high-quality images and permitting the decrease of cost toward the improvement in the temperature characteristics.

A further object of the present invention is to provide an electrophotographic, photosensitive member that permits power savings, decrease of tact time, and decrease of production cost in production of the electrophotographic, photosensitive member, and an image forming apparatus having the photosensitive member.

A further object of the present invention is to provide an electrophotographic, photosensitive member that can present high-quality images with fewer image defects of blank area or the like due to the film peeling off of the a-Si(H,X) deposited film and that can be produced at low cost, and an electrophotographic apparatus having the photosensitive member.

Another object of the present invention is to provide an electrophotographic apparatus incorporating a photoconductive member for electrophotography that always demonstrates stable, electrical, optical, and photoconductive properties, that suffers no deterioration in repetitive use, and that has excellent endurance.

According to the present invention, there is provided an electrophotographic, photosensitive member which is cylindrical and comprises a photosensitive layer comprising amorphous silicon provided on an electroconductive substrate and in which the thickness of the electroconductive substrate is not less than 0.1 mm but less than 2.5 mm, wherein the photosensitive layer is a layer formed by a plasma CVD method to induce a discharge at a discharge frequency of not less than 50 MHz nor more than 450 MHz, and an electrophotographic apparatus comprising the electrophotographic, photosensitive member.

According to the present invention, there is further provided an electrophotographic, photosensitive member which has a cylindrical shape and comprises a photosensitive layer comprising amorphous silicon provided on an electroconductive substrate, wherein the electroconductive substrate has a thickness of not less than 0.1 mm but less than 2.5 mm, and wherein the outside diameter of the cylinder is not less than 20 mm nor more than 60 mm, and an electrophotographic apparatus comprising the electrophotographic, photosensitive member.

#### BRIEF DESCRIPTION OF THE DRAWINGS

FIG. 1A is a schematic, perspective view of a photosensitive member and FIG. 1B is a schematic, sectional view of the photosensitive member;

FIG. 2 is a schematic, structural view for explaining an example of a deposition system;

FIG. 3 is a schematic, structural view for explaining an example of a production system for formation of deposited film;

FIG. 4 is a schematic, structural view for explaining an example of a deposition system;

FIG. 5A is a schematic, perspective view showing an example of a heater and FIG. 5B is a schematic, perspective view showing an example of application of the heater of FIG. 5A to a photosensitive member;

FIG. 6 is a schematic block diagram showing an example of a temperature regulating mechanism of the heater;

FIG. 7 is a schematic block diagram showing an example of another temperature regulating mechanism of the heater;

FIG. 8A and 8B are schematic, perspective views showing an example of a PTC heater;

FIG. 9 is a graph showing an example of surface temperature of the photosensitive member in a quiescent state (a static state);

FIG. 10 is a graph showing an example of surface temperature of the photosensitive member in a quiescent state (a static state);

FIG. 11 is a graph showing an example of surface temperature of the photosensitive member in a sheet pass state (a dynamic state);

FIG. 12 is a graph showing an example of surface temperature of the photosensitive member in a sheet pass state (a dynamic state); and

FIG. 13 is a schematic, structural view showing an example of the image forming apparatus.

#### DESCRIPTION OF THE PREFERRED EMBODIMENTS

The present invention is based on such a finding that the above problems including the film peeling off etc. were able to be solved even with the thin substrate by use of the drum-like metal substrate having a specific outside diameter as a support for the a-Si(H,X) deposited film, as a consequence of systematic, intensive and extensive studies and investigations from the viewpoints of adaptability and applicability of a-Si(H,X) to the photoconductive member used in the image forming member for electrophotography.

The drum-like metal substrate in the present invention is one having the thickness not less than 0.1 mm but less than 2.5 mm and the outside diameter not less than 20 mm nor more than 60 mm. With use of the drum-like metal substrate having the outside diameter not less than 20 mm nor more than 60 mm, even if the drum-like metal substrate is heated in the deposition system of the a-Si(H,X) film during the production of the photoconductive member or even if the drum-like metal substrate is heated during use as a photosensitive drum for electrophotography, the degree of thermal deformation of the drum-like metal substrate can be controlled to a sufficiently small level, so that the degree of the film peeling off of the a-Si(H,X) deposited film can be decreased to below a level in which no problem is posed in practical use, or to zero.

In the photosensitive member of the present invention, the electroconductive substrate is one having the thickness not less than 0.1 mm but less than 2.5 mm and the photoconductive member containing a-Si is made by the plasma CVD method to induce discharge at the discharge frequency not less than 50 MHz nor more than 450 MHz, whereby the degree of thermal deformation of the drum-like metal substrate can be suppressed to a sufficiently small level even if the drum-like metal substrate is heated in the a-Si(H,X) film deposition apparatus during the production of the photoconductive member or even if the drum-like metal substrate is heated during use as a photosensitive drum for electrophotography. Therefore, the degree of film peeling off of the a-Si(H,X) deposited film can be decreased to the level in which no problem is posed in practical use, or to zero. Further, deformation of the drum-like metal substrate due to stress of film can also be suppressed.

It is also preferable that the photosensitive member of the present invention have the layer structure as illustrated in FIG. 1B. A preferred composition of each layer will be described below.

##### [Charge injection inhibiting layer]

The charge injection inhibiting layer in the electrophotographic, photosensitive member of the present invention has a function to inhibit charge from being injected from the conductive support side into the photoconductive layer side when the electrophotographic, photosensitive member undergoes a charging process of a certain

polarity on its free surface, and also has a so-called polarity dependence not to demonstrate the function when it is subject to a charging process of the opposite polarity. In order to impart such functions, the inhibiting layer is made to contain a relatively larger amount of atoms for controlling the electroconductive property than the photoconductive layer. The atoms for controlling the electroconductive property, contained in the inhibiting layer, can be either the IIIb atoms or the Vb atoms. A content of the atoms for controlling the electroconductive property, contained in the inhibiting layer in the present invention, is properly determined as desired so as to accomplish the objects of the present invention effectively and it is desirable to determine the content preferably in the range of 10 to  $1\times 10^4$  atomic ppm, more preferably in the range of 50 to  $5\times 10^3$  atomic ppm, and most preferably in the range of  $1\times 10^2$  to  $1\times 10^3$  atomic ppm.

The hydrogen atoms and/or halogen atoms contained in the inhibiting layer compensate for dangling bonds existing in the layer so as to improve the quality of film. It is desirable to determine the content of the hydrogen atoms or halogen atoms or the content of the sum of the hydrogen atoms and halogen atoms in the inhibiting layer preferably in the range of 1 to 50 atomic %, more preferably in the range of 5 to 40 atomic %, and most preferably in the range of 10 to 30 atomic %.

It is desirable in the present invention to determine the thickness of the inhibiting layer preferably in the range of 0.1 to 5  $\mu\text{m}$  and most preferably in the range of 1 to 4  $\mu\text{m}$  in terms of capability of obtaining desired electrophotographic characteristics, the economical effect, and so on.

[Photoconductive layer]

The photoconductive layer in the electrophotographic, photosensitive member of the present invention needs to contain the hydrogen atoms or/and halogen atoms in the film. This is because they are necessary and indispensable for compensating for the dangling bonds of silicon atoms and for improving the quality of layer, particularly, for enhancing the photoconductive property and charge retaining characteristics. It is thus desirable to determine the content of the hydrogen atoms or halogen atoms or the total amount of the hydrogen atoms and halogen atoms in the range of 10 to 30 atomic % and more preferably in the range of 15 to 25 atomic % relative to the sum of the silicon atoms and the hydrogen atoms or/and halogen atoms. The amount of the hydrogen atoms or/and halogen atoms contained in the photoconductive layer can be controlled, for example, by controlling the temperature of the support, an introduced amount of the raw material for inclusion of the hydrogen atoms or/and halogen atoms into the reaction vessel, the discharge power, and so on.

It is preferable in the present invention to make the photoconductive layer contain the atoms for controlling the electroconductive property as occasion may demand. The atoms for controlling the electroconductive property can be those used for the inhibiting layer. It is desirable to determine the content of the atoms for controlling the electroconductive property present in the photoconductive layer, to be preferably in the range of  $1\times 10^{-2}$  to  $1\times 10^4$  atomic ppm, more preferably in the range of  $5\times 10^{-2}$  to  $5\times 10^3$  atomic ppm, and most preferably in the range of  $1\times 10^{-1}$  to  $1\times 10^3$  atomic ppm.

Further, in the present invention, it is effective to make the photoconductive layer contain carbon atoms, oxygen atoms, or nitrogen atoms. It is desirable to determine the content of the carbon atoms, oxygen atoms, or nitrogen atoms preferably in the range of  $1\times 10^{-5}$  to 10 atomic %, more preferably

in the range of  $1\times 10^{-4}$  to 8 atomic %, and most preferably in the range of  $1\times 10^{-3}$  to 5 atomic % relative to the sum of the silicon atoms, carbon atoms, oxygen atoms, and nitrogen atoms. The carbon atoms, oxygen atoms, or nitrogen atoms do not always have to be contained throughout the entire layer, but they may be distributed only in a part thereof or across the thickness (with variations in density).

It is desirable in the present invention to determine the thickness of the photoconductive layer properly taking into account the desired electrophotographic characteristics, the economical effect, and so on, and to determine the thickness preferably in the range of 10 to 50  $\mu\text{m}$ , more preferably in the range of 20 to 45  $\mu\text{m}$ , and most preferably in the range of 25 to 40  $\mu\text{m}$ .

[Surface protecting layer]

It is preferable in the present invention to further form the a-Si-based or a-C-based surface protecting layer on the photoconductive layer. This surface protecting layer has a free surface and is provided mainly for accomplishing the objects of the present invention in the moisture resistance, continuous and repetitive operation characteristics, dielectric strength, operating environment characteristics, and durability. In the present invention, because each of the amorphous materials forming the photoconductive layer and the surface protecting layer constituting the photoreceptive layer has the common component of silicon atoms, chemical stability is assured well at the stacking interface between the layers.

The surface protecting layer can be comprised of any a-Si-based or a-C-based material, and examples of preferred materials therefor are a-Si containing hydrogen atoms (H) and/or halogen atoms (X) and further containing carbon atoms (a-SiC:H,X), a-Si containing hydrogen atoms (H) and/or halogen atoms (X) and further containing oxygen atoms (a-SiO:H,X), a-Si containing hydrogen atoms (H) and/or halogen atoms (X) and further containing nitrogen atoms (a-SiN:H,X), a-Si containing hydrogen atoms (H) and/or halogen atoms (X) and further containing at least one of carbon, oxygen, and nitrogen (a-SiCON:H,X), and so on.

The content of an element or elements selected from carbon, nitrogen, and oxygen is preferably in the range of 30 atomic % to 90 atomic % relative to the sum of the silicon atoms and, the carbon atoms, nitrogen atoms, and/or oxygen atoms.

In the present invention, the surface protecting layer needs to contain hydrogen atoms or/and halogen atoms, and it is desirable to determine the hydrogen content normally in the range of 30 to 70 atomic %, preferably in the range of 35 to 65 atomic %, and most preferably in the range of 40 to 60 atomic % relative to the total amount of the component atoms. It is also desirable to determine the content of fluorine atoms normally in the range of 0.01 to 15 atomic %, preferably in the range of 0.1 to 10 atomic %, and most preferably in the range of 0.6 to 4 atomic %.

In the present invention, the surface protecting layer may further contain the atoms for controlling the conductivity type as occasion may demand.

It is desirable in the present invention to determine the thickness of the surface protecting layer normally in the range of 0.01 to 3  $\mu\text{m}$ , preferably in the range of 0.1 to 2  $\mu\text{m}$ , and most preferably in the range of 0.5 to 1  $\mu\text{m}$ . If the thickness of the layer is smaller than 0.01  $\mu\text{m}$  the surface protecting layer will be lost for the reason of wear or the like during use of the electrophotographic, photosensitive member. If the thickness is over 3  $\mu\text{m}$  degradation will occur in the electrophotographic characteristics, such as increase of the residual potential and the like.

The atoms for controlling the conductivity type in the present invention, for example, specific examples of the IIIb atoms include B (boron), Al (aluminum), Ga (gallium), In (indium), Tl (thallium), and so on, among which B, Al, and Ga are particularly suitable. Specific examples of the Vb atoms are P (phosphorus), As (arsenic), Sb (antimony), Bi (bismuth), and so on, among which P and As are particularly suitable.

The IIIb atoms or the Vb atoms can be structurally introduced by introducing the raw material for introduction of the IIIb atoms or the raw material for introduction of the Vb atoms in a gas state, together with the other gases, into the reaction vessel on the occasion of formation of the layer. The raw material for introduction of the IIIb atoms or the raw material for introduction of the Vb atoms is desirably a gaseous material at ordinary temperature and ordinary pressure or a material that can be readily gasified at least under the film-forming conditions. Specific examples of the raw material for introduction of the IIIb atoms, e.g. for introduction of boron atoms, include boron hydrides such as  $B_2H_6$ ,  $B_4H_{10}$ ,  $B_5H_9$ ,  $B_5H_{11}$ ,  $B_6H_{10}$ ,  $B_6H_{12}$ , and  $B_6H_{14}$ , boron halides such as  $BF_3$ ,  $BCl_3$ , and  $BBr_4$ , and so on. Further examples include  $AlCl_3$ ,  $GaCl_3$ ,  $Ga(CH_3)_3$ ,  $InCl_3$ ,  $TiCl_3$ , and so on. Specific examples of the raw material effectively used for introduction of the Vb atoms, e.g. for introduction of phosphorus atoms, are phosphorus hydrides such as  $PH_3$ ,  $P_2H_4$  and the like, phosphorus halides such as  $PH_4I$ ,  $PF_3$ ,  $PF_5$ ,  $PCl_3$ ,  $PCl_5$ ,  $PBr_3$ ,  $PBr_5$ ,  $PI_3$ , and the like, and so on. Further examples of the raw material that can be effectively used as a starting substance for introduction of the Vb atoms include  $AsH_3$ ,  $AsF_3$ ,  $AsCl_3$ ,  $AsBr_3$ ,  $AsF_5$ ,  $SbH_3$ ,  $SbF_3$ ,  $SbF_5$ ,  $SbCl_3$ ,  $SbCl_5$ ,  $BiH_3$ ,  $BiCl_3$ ,  $BiBr_3$ , and so on. These raw materials for introduction of the atoms for controlling the conductivity type may be used as diluted with  $H_2$  and/or He if necessary.

Substances that can be used as an Si-supplying gas in the present invention are gaseous or gasifiable silicon hydrides (silanes) such as  $SiH_4$ ,  $Si_2H_6$ ,  $Si_3H_8$ ,  $Si_4H_{10}$ , etc. which can be used effectively in the present invention. Preferred materials are  $SiH_4$  and  $Si_2H_6$  in terms of ease to handle during formation of the layer, high Si supply efficiency, and so on.

The layer can also be formed by further mixing a desired amount of  $H_2$  and/or He, or a gas of a silicon compound containing hydrogen atoms into the above-stated gases in order to structurally introduce the hydrogen atoms into each layer to be formed, further facilitate control of the rate of hydrogen atoms introduced, and obtain desired film characteristics to accomplish the objects of the present invention. Each gas may be not only a single species, but also a mixture of plural species at a predetermined mixture ratio.

The optimum range of flow rate of  $H_2$  and/or He used as a dilution gas is properly selected according to the design of the layer, and it is desirable to control  $H_2$  and/or He normally in the range of 3 to 20 times, preferably in the range of 4 to 15 times, and most preferably in the range of 5 to 10 times the flow rate of the gas for supply of Si.

Preferred examples of materials effectively used as the source gas for supply of halogen atoms in the present invention include gaseous or gasifiable halogen compounds such as halogen gases, halogenides, interhalogen compounds containing halogen, silane derivatives substituted by halogen, and so on. In addition, further materials effectively used are gaseous or gasifiable silicon hydride compounds containing halogen atoms, components of which are silicon atoms and halogen atoms. Specific examples of the halogen compounds that can be preferably used in the present invention are fluorine gas ( $F_2$ ), and the interhalogen com-

pounds such as  $BrF$ ,  $CIF$ ,  $CIF_3$ ,  $BrF_3$ ,  $IF_3$ ,  $IF_7$ , and so on. Preferred examples of the silicon compounds containing halogen atoms, which are so called the silane derivatives substituted by halogen atoms, are, specifically, silicon fluorides, for example, such as  $SiF_4$ ,  $Si_2F_6$ , and so on.

Substances that can be effectively used as a gas for supply of carbon are gaseous or gasifiable hydrocarbons such as  $CH_4$ ,  $C_2H_6$ ,  $C_3H_8$ ,  $C_4H_{10}$ , etc. among which preferred hydrocarbons are  $CH_4$  and  $C_2H_6$  in terms of ease to handle during production of the layer, the high C supply efficiency, and so on.

Substances that can be effectively used as a gas for supply of nitrogen or oxygen are gaseous or gasifiable compounds such as  $NH_3$ ,  $NO$ ,  $N_2O$ ,  $NO_2$ ,  $O_2$ ,  $CO$ ,  $CO_2$ ,  $N_2$ , and so on.

The atoms contained in each layer may be uniformly distributed throughout the layer, or may be contained throughout the layer in the layer thickness direction but nonuniformly distributed. In either case, it is, however, necessary to distribute the atoms uniformly and all over in the in-plane directions parallel to the surface of the support, from the aspect of uniforming the characteristics in the in-plane directions.

The optimum range of the gas pressure inside the reaction vessel is also properly selected according to the layer design and the pressure is determined normally in the range of  $1 \times 10^{-4}$  to 10 Torr, preferably in the range of  $5 \times 10^{-4}$  to 5 Torr, and most preferably in the range of  $1 \times 10^{-3}$  to 1 Torr.

The optimum range of the discharge power is also properly selected according to the layer design, and it is desirable to set the discharge power per flow rate of the gas for supply of Si normally in the range of 2 to 7 times, preferably in the range of 2.5 to 6 times, and most preferably in the range of 3 to 5 times.

The optimum range of the temperature of the support is also properly selected according to the layer design and it is desirable normally to determine the temperature preferably in the range of 50 to 500°C. and more preferably in the range of 200 to 350°C.

In the present invention, the above-stated ranges can be listed as desired numerical ranges of the mixture ratio of the source gases for formation of each layer, the gas pressure, the temperature of the support, and the discharge power, but these conditions, normally, cannot be determined independent of each other. It is thus desirable to determine the optimum values, based on mutual and organic relation so as to form the deposited film with desired characteristics.

The photosensitive member for electrophotography of the present invention described above is formed by a vacuum deposited film forming method. Specifically, it can be formed by various thin film deposition methods, for example, such as the glow discharge methods (ac discharge CVD methods including low-frequency CVD methods, high-frequency CVD methods, microwave CVD methods, and so on, or dc discharge CVD methods, etc.), sputtering methods, vacuum evaporation methods, ion plating methods, photo CVD methods, thermal CVD methods, and so on. These thin film deposition methods are properly selected and employed depending upon factors including the production conditions, degrees of loads under capital investment on production facilities, production scale, desired characteristics for the electrophotographic, photosensitive member produced, and so on. The glow discharge methods are preferably used, because it is relatively easy to control the conditions for production of the electrophotographic, photosensitive member with the desired characteristics, and the high-frequency glow discharge methods using the power-supply frequency in the RF band or in the VHF band

are particularly preferred. In the present invention, the deposited film is formed, for example, by the high-frequency plasma CVD method at the power-supply frequency in the VHF band, not less than 50 MHz nor more than 450 MHz.

The apparatus and forming method will be detailed below.  
<Production apparatus>

FIG. 3 is a schematic, structural view showing an example of the production apparatus by the RF-CVD method.

In FIG. 3, reference numeral 3100 designates a deposition device and 3200 a gas supply device which supplies the source gases and/or a dilution gas necessary for formation of the deposited film and the like.

A deposition chamber is composed of a wall 3111, a base plate 3121, a gate valve 3120, and an insulator 3122 and has gas inlet pipes 3114 and a heater 3113 for heating the support 3112 in the space inside the chamber. The space inside the deposition chamber is connected via an exhaust valve 3118 to an exhaust pump 3117 by an exhaust pipe 3119. The exhaust pipe has a vacuum gage 3124 and an atmosphere communication valve 3123 between the exhaust valve 3118 and the deposition chamber. Reference numeral 3115 denotes an RF power supply, and the wall 3111 serves as one electrode while the support 3112 as the other electrode in this example.

A gas supply pipe 3116 for the gases supplied from the gas supply device 3200 is connected to the gas inlet pipes 3114. The source gases including the dilution gas are enclosed in respective bombs 3221 to 3226, and they are supplied from valves 3231 to 3236 through inflow valves 3241 to 3246, mass flow controllers 3211 to 3216, and outflow valves 3251 to 3256 and through a connection valve 3260 to the deposition device side. Reference numerals 3261 to 3266 represent pressure regulators.

Next described is an example of the method for producing the electrophotographic, photosensitive member for electrophotography formed by the high-frequency plasma CVD (VHF-PCVD method) process using the frequency in the VHF band.

An apparatus for producing the electrophotographic, photosensitive member for electrophotography by the VHF-PCVD process can be constructed by connecting the deposition device illustrated in FIG. 4, instead of the deposition device by the RF-PCVD method in the production apparatus shown in FIG. 3, to the source gas supply device (3200).

This apparatus is generally constructed of a depressurizable reaction vessel 4111 of the vacuum hermetic structure, the source gas supplying device 3200, and an evacuation system (not illustrated) for depressurizing the inside of the reaction vessel 4111. Inside the reaction vessel 4111 there are provided electroconductive supports 4112, heaters 4113 for heating the supports, source gas inlet pipes (not illustrated), and an electrode 4115, and a high-frequency matching box 4116 is further connected to the electrode 4115. The space inside the reaction vessel 4111 is connected to an unrepresented diffusion pump through an exhaust pipe 4121. Numeral 4120 stands for motors for rotating the associated supports 4112.

The source gas supplying device 3200 is constructed of bombs of source gases such as SiH<sub>4</sub>, GeH<sub>4</sub>, H<sub>2</sub>, CH<sub>4</sub>, B<sub>2</sub>H<sub>6</sub>, PH<sub>3</sub>, etc., valves, and mass flow controllers, a bomb of each source gas being connected via a valve to the gas inlet pipes (not illustrated) in the reaction vessel 4111. The space surrounded by the conductive supports 4112 creates a discharge space 4130.

Formation of the deposited film in this apparatus by the VHF-PCVD method is carried out as follows.

First, the conductive supports 4112 are set in the reaction vessel 4111, the supports 4112 are rotated by the driving

units 4120, and the inside of the reaction vessel 4111 is evacuated through the exhaust pipe 4121 by the unrepresented evacuation system (for example, a diffusion pump), thereby adjusting the pressure inside the reaction vessel to not more than  $1 \times 10^{-7}$  Torr. Next, the temperature of the conductive supports 4112 is raised to and maintained at a predetermined temperature in the range of 50° C. to 500° C. by the heaters 4113 for heating the supports.

For letting the source gases for formation of the deposited film into the reaction vessel, after it is confirmed that the valves of the gas bombs and the leak valve (not illustrated) of the reaction vessel are closed and that the inflow valves 3241-3246, the outflow valves 3251-3256, and the auxiliary valve 3260 are opened, the main valve (not illustrated) is first opened to evacuate the inside of the reaction vessel and gas pipes. When the reading of the vacuum gage (not illustrated) then reaches about  $5 \times 10^{-6}$  Torr, the auxiliary valve and outflow valves are closed.

After that, each gas is introduced from the corresponding gas bomb with opening the associated valve and the pressure of each gas is regulated to 2 kg/cm<sup>2</sup> by the pressure regulator 3261-3266. Then the inflow valve is gradually opened to introduce each gas into the mass flow controller.

After completion of the preparation for deposition as described above, formation of each layer is carried out.

When the conductive supports reach the predetermined temperature, necessary valves out of the outflow valves and the auxiliary valve are gradually opened to introduce prescribed gases from the corresponding gas bombs through the gas inlet pipes (not illustrated) into the discharge space in the reaction vessel. Then the flow of each source gas is adjusted to a predetermined flow rate by the corresponding mass flow controller. On that occasion, the degree of valve opening of the main valve (not illustrated) is adjusted with observing the vacuum gage (not illustrated) so that the pressure inside the discharge space becomes a predetermined pressure of not more than 1 Torr.

Deposition of each layer is carried out as follows. The VHF power supply (not illustrated), for example, of the frequency 500 MHz is set to a desired power, and the VHF power is introduced via the matching box 4116 to the discharge space 4130 to induce glow discharge. In the discharge space 4130 surrounded by the supports 4112, the source gases introduced are thus excited and dissociated by discharge energy, whereby a predetermined deposition film is formed on the supports 4112. At this time, the output of the heaters 4113 for heating the supports is adjusted at the same time as the introduction of the VHF power to change the temperature of the conductive supports 4112 to a desired value. On this occasion, the supports are rotated at a desired rotation rate by the motors 4120 for rotation of the supports in order to uniform the formation of layer.

After completion of formation of the film in a desired film thickness, the supply of the VHF power is terminated and the outflow valves are closed to stop the inflow of the gases into the reaction vessel, thus completing the formation of the desired layer.

The like operation is repeated several times, if necessary, thereby forming the electrophotographic, photosensitive member in desired layer structure.

It is needless to mention that all the other outflow valves than those of the necessary gases are closed in formation of each layer and, in order to prevent each gas from remaining inside the reaction vessel or inside the pipes from the outflow valves to the reaction vessel, an operation for once evacuating the inside of the system to a high vacuum is carried out according to the necessity by closing the outflow

valves, opening the auxiliary valve, and fully opening the main valve (not illustrated).

It is needless to mention that the above-stated gas species and valve operations are modified according to the production conditions of each layer.

The heating means for the conductive substrates can be any heat-generating member prepared in a vacuum specification and, more specifically, they can be selected from electric resistance heat-generating members such as winding heaters of sheath heaters, sheet-like heaters, ceramic heaters, and so on, heat-radiating lamp heat-generating members such as halogen lamps, infrared lamps, and so on, heat-generating members by heat exchange means using liquid, gas, or the like as a heat medium, and so on. A material for the surface of the heating means can be selected from metals such as stainless steel, nickel, aluminum, copper, and the like, ceramics, heat-resistant polymers, and so on. In addition thereto, another applicable method is a method in which a vessel dedicated for heating is provided in addition to the reaction vessel, the conductive supports are heated in the dedicated vessel, and thereafter the conductive supports are transferred into the vacuum in the reaction vessel, for example.

It is also desirable to determine the pressure of the discharge space, particularly, in the VHF-PCVD method preferably in the range of not less than 1 mTorr nor more than 500 mTorr, more preferably in the range of not less than 1 mTorr nor more than 300 mTorr, and most preferably in the range of not less than 1 mTorr nor more than 100 mTorr.

The size and shape of the electrode **4115** provided in the discharge space in the VHF-PCVD method can be any size and shape as long as they do not disorder the discharge, but a preferred electrode is a cylindrical one having the diameter of not less than 1 mm nor more than 10 cm in practical use. At this time, the length of the electrode can also be set to an arbitrary value as long as it is such a length as to realize uniform application of the electric field to the conductive supports.

The material for the electrode **4115** can be any material as long as the surface is electrically conductive. The material is normally selected, for example, from metals such as stainless steel, Al, Cr, Mo, Au, In, Nb, Te, V, Ti, Pt, Pb, Fe, and so on, alloys thereof, glasses or ceramics with a surface undergoing an electroconductive treatment, and so on.

The electrophotographic, photosensitive member produced by the method of the present invention can be used not only in the electrophotographic copiers, but also in applications of electrophotography, including laser beam printers, CRT printers, LED printers, liquid crystal printers, laser engraving machines, and so on.

Next described is the electrophotographic apparatus incorporating the photosensitive member of the present invention.

#### <Electrophotographic apparatus>

It is known heretofore that in the electrophotographic apparatus making use of the corona charging, ozone products are attached to the surface of the photosensitive member to cause image unfocussing, particularly, at high humidity. In the case of the photoconductive members having the surface relatively easy to wear like organic photoconductors (OPCs), it is easy to wear and remove the ozone products etc. formed on the surface by a polishing means or the like, but the polishing effect, if too high, will degrade the function as a photosensitive member to shorten the lifetime. In the case of the surface insulating layer of the CdS photosensitive member used in the amorphous photosensitive members (hereinafter referred to as a-Si photosensitive

members) or in the NP method, the surface layer is very hard and the ozone oxides etc. formed on the surface are resistant to wear and removal in certain cases.

It is thus the practice to provide a heater inside and near the photosensitive member to heat the surface of the photosensitive member to the temperature of about 35 to 45° C. This heating of the photosensitive member is carried out for various purposes, but a principal purpose is to prevent and remove the image unfocussing occurring at high humidity. 10 This is for the following reason. The ozone evolving in the corona charger chemically deteriorates the surface of the photosensitive member to make the hydrophilic groups (—OH etc.) and the like, and the surface becomes apt to absorb moisture. This causes a phenomenon of lateral flow 15 of surface potential which is fatal to electrophotography. Therefore, the surface is heated to remove water. Since the substances of NO<sub>x</sub> etc. produced by ozone attach to the surface of the photosensitive member and absorb moisture similarly, the principal purpose is to heat the surface to 20 remove water similarly.

The heating means can be a hot air blow or the like, but the dominating heating means is heating with an electric heater from the inside of the photosensitive member. It was the conventional practice to employ a temperature-controlling method with a rod heater disposed in a shaft for supporting the photosensitive member, as a rotational shaft of the photosensitive member, but it is recently common practice, particularly in the a-Si photosensitive members, to employ a method of placing a sheet-like heater on the inside 25 surface of the photosensitive member in order to enhance the temperature control accuracy for control of the surface temperature of the photosensitive member and eliminate temperature irregularities across the entire surface of the photosensitive member.

30 The conventional heating means will be described specifically.

FIG. 5A is a schematic, perspective view showing a curved state of a flat sheet heater **501A** for the photosensitive member before mounted and FIG. 5B is a schematic, perspective view showing a state in which the flat sheet heater **501A** for the photosensitive member is mounted with a clearance **503** inside the drum of the photosensitive member. There are commonly used heaters for the photosensitive member, which are generally classified under the rod-like 35 type in which the heater is disposed without contact with the inside surface of the photosensitive member, which is not illustrated, and the sheet-like type in which the heater is in contact with the inside surface of the photosensitive member, as in the figure. The latter sheet-like type has higher 40 temperature control accuracy.

45 FIG. 6 and FIG. 7 show examples of blocks for control of temperature.

In FIG. 6, reference numeral **601** designates a heater for photosensitive member, **602** an AC power supply for supply of power, **603** a thermistor for temperature feedback, and **604** a control circuit for controlling switching of on/off or several steps of power supply to the heater according to the resistance of the thermistor **603**. Wave lines in the figure indicate the border between the main body of the electrophotographic apparatus and the photosensitive member unit, which normally contact with each other through a slip ring or the like. Since the thermistor **603** has such a property as to turn into a low resistance at high temperature, the temperature is fed back to the control circuit to effect the 50 temperature control.

55 In FIG. 7, reference numeral **701** designates a heater for the photosensitive member, **702** an AC power supply for

supply of power, and 703 a thermoswitch for control of temperature. Wave lines in the figure indicate the border between the main body of the electrophotographic apparatus and the photosensitive member unit, which normally contact with each other through a slip ring or the like. The thermoswitch 703 is connected so as to become off at high temperature, thereby effecting the temperature control. The temperature for off of the thermoswitch is a specific property of the thermoswitch.

The control with the thermistor as illustrated in FIG. 6 permits higher temperature control accuracy because of the structure. Particularly, in the case of the a-Si photosensitive members, the potentials have the temperature dependence of 1 to 6 V/deg as to the dark area potential (300 to 500 V) and the temperature dependence of 1 to 3 V/deg as to the light area potential (50 to 200 V) and thus the accuracy of about  $\pm 1^\circ \text{C}$ . is sometimes required for the control of the heating temperature. In this case the configuration of FIG. 6 is more preferred.

This accuracy is implemented with the photosensitive member alone or in a static state in which the photosensitive member is in quiescent operation even if set in the electrophotographic apparatus, but the temperature of the photosensitive member is greatly influenced by the room temperature and the copy mode in a dynamic state, i.e., in a state of sheet pass as actually used in the electrophotographic apparatus. Namely, a quantity of heat transferred from the photosensitive member to the sheet during the sheet pass affects the temperature of sheet and the temperature of the sheet is affected by the room temperature and the copy mode (i.e., whether the sheet about to be used for copy is a sheet newly supplied from the outside of the electrophotographic apparatus or a sheet after pass through a fixing device as in the case of double-side copy, multiple copy, or the like). Since the quantity of heat transferred from the photosensitive member to the sheet is also affected by the frequency of contact between the sheet and the photosensitive member, the influence of the copy mode (whether single side or double side, the set number of copies, the sheet size [size and thickness], etc.) is significant. In order to control the temperature of the photosensitive member at a constant value in the dynamic state, it is thus necessary to supply a much higher power than for the temperature equilibrium state to the heater, so as to increase the response.

When the power supply is increased, the conventional methods, however, could suffer temperature unevenness for the two reasons below in certain cases.

The first reason is the issue of the shape. In the case of the method in which the flat sheet heater is curved so as to be in close fit to the inside surface of the cylindrical, photosensitive member, the temperature response is poor at the seam part of the heater and there sometimes arises a temperature difference between the seam part and the heater part. One method for overcoming it is use of a seamless heater.

The second reason is the issue of the control method. In the case of the control method to effect switching with the circuit using the thermistor, though depending upon the temperature detection position and the control circuit, there is such a general tendency that overshoots and temperature control ripples increase with increase of power. In order to reduce them, the control circuit became expensive and the temperature unevenness had to be conceded to some extent, taking practical cost into consideration.

It is then conceivable to employ a PTC (positive temperature coefficient) heater (self-temperature-control heater) whose resistance has a temperature dependence. The PTC

heater is a heater utilizing such a property of the resistor itself as to increase the resistance at high temperature and being capable of controlling the temperature of the resistor so as to be constant. Therefore, the PTC heater needs no temperature control circuit and theoretically suffers no overshoots or ripples.

The PTC heater is a heater self-controlled at an appropriate temperature because of the PTC characteristics of the PTC resistor between electrodes. An example of the known PTC heater is a sheet-like heat-generating member in which a heat-generator layer and electrodes are laminated through a thermoadhesive resin with respect to an insulating layer of a film shape by a laminating device or by heating and pressing to bond them into an integral form. There are various configurations depending upon the needs such as high temperature, high power, and so on, including the configurations composed of a pair of electrodes as described in Japanese Patent Publications No. 57-43995 and No. 55-40161, and their fundamental structure is substantially the same.

It is, therefore, considered that use of the PTC heater in the seamless structure is extremely effective means in the electrophotographic apparatus that has to be controlled with large power, as described previously.

As described above, the drum-like metal substrate can be formed in the thickness of not less than 0.1 mm but less than 2.5 mm, whereby the production cost can be curtailed drastically.

When the heater is used in the drum-like metal substrate having the thickness of not less than 0.1 mm but less than 2.5 mm, the temperature control can be achieved with high accuracy, because the temperature gradient is small between the heater and the surface of the photosensitive member.

Further, because the use of the PTC heater in the seamless structure permits input of much higher power than for the temperature equilibrium state, the response is increased to make quick temperature increase possible and the temperature control can be performed without the overshoots nor the temperature-control ripples even in the dynamic state with sheet pass.

When the drum-like metal substrate used is one having the outside diameter not less than 20 mm nor more than 60 mm, the degree of thermal deformation of the drum-like metal substrate can be suppressed to a sufficiently small level even if the drum-like metal substrate is heated during production of the photoconductive member and during use as a photosensitive drum for electrophotography. Therefore, the degree of film peeling off of the a-Si(H,X) deposited film can be controlled to a level in which no problem is posed in the practical use, or to zero. In addition, the thickness of the drum-like metal substrate can be made not less than 0.1 mm but less than 2.5 mm, whereby the production cost can be curtailed drastically.

FIG. 13 is a schematic view of image forming apparatus for explaining an example of the image forming apparatus.

Around the photosensitive member 101 for the image forming apparatus utilizing the electrophotographic method (hereinafter referred to simply as "photosensitive member"), which rotates in the direction of arrow X, there are a primary charger 102, an electrostatic latent image forming section 103, a developing unit 104, a transfer sheet supply system 105, a transfer charger 106a, a separation charger 106b, a cleaner 107, a conveying system 108, a charge-eliminating light source 109, etc., which are disposed in the stated order clockwise in the figure. The photosensitive member 101 may be subjected to the temperature control with a sheet-like inside heater 125 as occasion demands.

The photosensitive member 101 is uniformly charged in the surface thereof with the primary charger 102 and is exposed to light according to the necessity at the electrostatic latent image forming section 103 to form an electrostatic latent image thereon.

This electrostatic latent image is developed into a toner image by a developing sleeve of the developing unit 104 coated with a developer (toner).

On the other hand, a transfer sheet P is supplied while guided by transfer sheet guide 119 of the transfer sheet supply system 105 and adjusted at the tip by registration rollers 122, and the toner image formed on the surface of the photosensitive member 101 is transferred onto the transfer sheet P with the transfer charger 106a. The transfer sheet P is separated from the photosensitive member 101 by the separation charger 106b and/or a separating means such as a claw (not illustrated) or the like. The transfer sheet is conveyed via the conveying system 108 into a fixing device 123 and the toner image on the surface thereof is fixed by fixing rollers 124 in the fixing unit 123. After that, the transfer sheet is discharged out of the image forming apparatus.

On the other hand, the surface of the photosensitive member 101 after the transfer of the toner image is processed by removing attached substances such as the residual toner, paper powder, etc. from the surface by a cleaning blade 120, a cleaning roller (or brush) 121 or the like in the cleaning device 107, and is then subjected to the next image formation.

## EXAMPLES

The present invention will be described in further detail with examples thereof, but it is noted that the present invention is by no means intended to be limited to these examples.

### Example 1

Using the production system of the photoconductive member for electrophotography illustrated in FIG. 2, the a-Si:H deposited film was formed under the below conditions on each of drum-like substrates of aluminum respectively having different outside diameters of 10 mm, 20 mm, 30 mm, 60 mm, 80 mm, and 108 mm and different thicknesses of 0.05 mm, 0.10 mm, 0.50 mm, 1.00 mm, 1.50 mm, 2.00 mm, 2.50 mm, 3.00 mm, 3.50 mm, and 5.00 mm, according to the glow discharge decomposition method detailed previously.

Temperature of drum-like substrate: 250° C.

Internal pressure inside the deposition chamber during formation of deposited film: 0.03 Torr

Discharge frequency: 13.56 MHz

Forming rate of deposited film: 20 Å/sec

Discharge power: 0.18 W/cm<sup>2</sup>

Thickness: 20 µm

The states of film peeling off of the electrophotographic, photosensitive drums thus obtained were observed and thereafter each of these photosensitive drums was set in a copying machine for tests modified for the tests to perform formation of image. The images were evaluated in order to indicate the influence of the film peeling off. The results are shown in Table 1.

TABLE 1

| Thickness | Film peeling off | Outside diameter |    |    |    |    |     |
|-----------|------------------|------------------|----|----|----|----|-----|
|           |                  | 10               | 20 | 30 | 60 | 80 | 108 |
| 10        | 0.05             | —                | —  | —  | —  | —  | —   |
|           | 0.10             | ○                | ○  | Δ  | Δ  | x  | x   |
|           | 0.50             | ○                | ○  | ○  | Δ  | x  | x   |
|           | 1.00             | ○                | ○  | ○  | Δ  | x  | x   |
|           | 1.50             | ○                | ○  | ○  | ○  | Δ  | x   |
|           | 2.00             | ○                | ○  | ○  | ○  | Δ  | x   |
|           | 2.50             | ○                | ○  | ○  | ○  | ○  | Δ   |
|           | 3.00             | ○                | ○  | ○  | ○  | ○  | ○   |
|           | 3.50             | ○                | ○  | ○  | ○  | ○  | ○   |
|           | 5.00             | ○                | ○  | ○  | ○  | ○  | ○   |

Criteria for evaluation:

○ very good,

○ good,

Δ practically acceptable,

x possibly problematic in practical use,

— unmeasurable

Criteria for evaluation: ○ very good, ○ good, Δ practically acceptable, x possibly problematic in practical use, —unmeasurable

The photosensitive drums of the substrate 0.05 mm thick suffered film peeling off during the deposition or during the measurement because of their insufficient strength and the measurement was impossible therewith.

It was confirmed that the film peeling off tended to decrease with increasing thickness. On the other hand, it was a new finding that the film peeling off tended to decrease with decreasing outside diameter.

Using the photosensitive drums of the outside diameter of 80 mm and 108 mm, the roundness was measured for the photosensitive drums of the thickness of 1.5 mm and 2.0 mm, and there was a difference of approximately 100 µm between the most depressed part and the most projecting part. In the case of the photosensitive drums of the thickness of 2.5 mm and 3.0 mm and the photosensitive drums of the outside diameter of 30 mm and 60 mm, the difference was about 30 µm. In the case of the photosensitive drums of the thickness of 3.5 mm and 5.0 mm, the difference was 10 to 20 µm. The evaluation results of roundness are shown in Table 2.

TABLE 2

| Thickness | Roundness | Outside diameter |    |    |    |    |     |
|-----------|-----------|------------------|----|----|----|----|-----|
|           |           | 10               | 20 | 30 | 60 | 80 | 108 |
| 50        | 0.05      | —                | —  | —  | —  | —  | —   |
|           | 0.10      | ○                | ○  | Δ  | Δ  | x  | x   |
|           | 0.50      | ○                | ○  | ○  | Δ  | x  | x   |
|           | 1.00      | ○                | ○  | ○  | Δ  | x  | x   |
|           | 1.50      | ○                | ○  | ○  | ○  | Δ  | x   |
|           | 2.00      | ○                | ○  | ○  | ○  | ○  | x   |
|           | 2.50      | ○                | ○  | ○  | ○  | ○  | Δ   |
|           | 3.00      | ○                | ○  | ○  | ○  | ○  | ○   |
|           | 3.50      | ○                | ○  | ○  | ○  | ○  | ○   |
|           | 5.00      | ○                | ○  | ○  | ○  | ○  | ○   |

Criteria for evaluation:

○ very good,

○ good,

Δ practically acceptable,

x possibly problematic in practical use,

— unmeasurable

Criteria for evaluation: ○ very good, ○ good, Δ practically acceptable, x possibly problematic in practical use, —unmeasurable

With the photosensitive members of the thin conductive substrate less than 2.5 mm, film peeling off levels of those

having the outside diameter not more than 60 mm were substantially equivalent to those of the photosensitive members of the thick photoconductive substrate not less than 2.5 mm.

#### Example 2

Using the PTC heater of a seamless cylinder shape and a flexible type to be set in close fit to the inside surface of the photosensitive member, as illustrated in FIGS. 8A and 8B, without use of the temperature control circuit, several types of photosensitive members having different thicknesses of the conductive substrate and different outside diameters of the cylinder were prepared and set in the test machine. Then the heater was activated with the optimum power according to the heat capacity of the photosensitive member and time changes of temperature were measured in a static state in which the temperature of the photosensitive member was controlled to 45° C., after the start of power supply to the heater. FIG. 9 shows an example of the results of the measurement. The determination results are shown in Table 3.

TABLE 3

| Static test (PTC) | Outside diameter |    |    |    |    |     |
|-------------------|------------------|----|----|----|----|-----|
|                   | 10               | 20 | 30 | 60 | 80 | 108 |
| Thickness         | 0.05             | —  | —  | —  | —  | —   |
|                   | 0.10             | —  | ○  | ○  | ○  | ○   |
|                   | 0.50             | —  | ○  | ○  | ○  | ○   |
|                   | 1.00             | —  | ○  | ○  | ○  | ○   |
|                   | 1.50             | —  | ○  | ○  | ○  | ○   |
|                   | 2.00             | —  | ○  | ○  | ○  | ○   |
|                   | 2.50             | —  | ○  | ○  | ○  | ○   |
|                   | 3.00             | —  | ○  | ○  | ○  | ○   |
|                   | 3.50             | —  | ○  | ○  | ○  | ○   |
|                   | 5.00             | —  | ○  | ○  | ○  | ○   |

Criteria for evaluation:  
 ○ very good,  
 ○ good,  
 — unmeasurable

Criteria for evaluation: ○ very good, ○ good,  
 —unmeasurable

The photosensitive drums of the substrate 0.05 mm thick suffered film peeling off during the deposition or during the measurement because of their insufficient strength and the measurement was impossible therewith.

FIG. 8A shows a shape of the heater for the photosensitive member before mounted and FIG. 8B shows a shape of the heater for the photosensitive member after mounted. During detachment or attachment, part of the heater is deformed, as illustrated in FIG. 8A, so as to decrease the substantial outside diameter. When mounted in the photosensitive member, the heater returns into the cylindrical shape by its restoring force so as to go into close fit to the inside surface of the photosensitive member. In order to realize it, the outside diameter of the heater is set equal to the inside diameter of the photosensitive member.

A typical example of the actual measurement is as shown in FIG. 9. Almost the same tendency was observed at all measured portions on the photosensitive member. When the temperature was increased quickly with large power, there appeared no temperature difference depending upon locations upon switching nor time changes (temperature control ripples) of temperature at the measured portions.

As shown in Table 3, the good results were obtained for all the samples with little dependence on the outside diameter by using the optimum power according to the heat

capacity of the photosensitive member. The results were better, particularly, with the samples of the thickness less than 2.5 mm.

#### Comparative Example 1

Using the temperature control circuit as illustrated in FIG. 6 and also using the heater of the type with a seam in which the flat sheet heater was curved so as to closely fit the inside surface of the photosensitive member, as illustrated in FIGS. 5A and 5B, and the heater of the seamless cylinder shape and of the flexible type to closely fit the inside surface of the photosensitive member, several types of photosensitive members having different thicknesses of the conductive substrate and different outside diameters of the cylinder were prepared and set in the test machine. Then the heater was activated with the power of Example 2 according to the heat capacity of the photosensitive member and time changes of temperature were measured in a static state in which the temperature of the photosensitive members was controlled to 45° C., after the start of power supply to the heater. FIG. 10 shows an example of the results of the measurement. The determination results are shown in Table 4.

TABLE 4

| 25        | Static test (conventional) | Outside diameter |    |    |    |    |     |
|-----------|----------------------------|------------------|----|----|----|----|-----|
|           |                            | 10               | 20 | 30 | 60 | 80 | 108 |
| Thickness | 0.05                       | —                | —  | —  | —  | —  | —   |
|           | 0.10                       | —                | ○  | ○  | ○  | ○  | ○   |
|           | 0.50                       | —                | ○  | ○  | ○  | ○  | ○   |
|           | 1.00                       | —                | ○  | ○  | ○  | ○  | ○   |
|           | 1.50                       | —                | ○  | ○  | ○  | ○  | ○   |
|           | 2.00                       | —                | ○  | ○  | ○  | ○  | ○   |
|           | 2.50                       | —                | ○  | ○  | ○  | ○  | ○   |
|           | 3.00                       | —                | ○  | ○  | ○  | ○  | ○   |
|           | 3.50                       | —                | ○  | ○  | ○  | ○  | ○   |
|           | 5.00                       | —                | ○  | ○  | ○  | ○  | ○   |

Criteria for evaluation:  
 ○ very good,  
 ○ good,  
 Δ practically acceptable,  
 — unmeasurable

Criteria for evaluation: ○ very good, ○ good, Δ practically acceptable, —unmeasurable

The photosensitive drums of the substrate 0.05 mm thick suffered film peeling off during the deposition or during the measurement because of their insufficient strength and the measurement was impossible therewith.

In FIG. 10, in the case of the heater of the type with the seam, the temperature changes were as indicated by the solid line at a portion which was not the seam of the heater and as indicated by the dashed line at the seam portion of the heater. There was thus a large temperature difference between them upon switching. On the other hand, in the case of the heater of the type without the seam, the temperature changes were as indicated by the solid line at all the measured portions, and there was no temperature difference depending upon locations upon switching. However, there appeared time changes of temperature (temperature control ripples) at the measured portions.

Even with the heaters of these types which posed no practical problem under the conventional, practical use conditions, the tendencies as described above became more prominent, particularly, with the thick samples, as shown in Table 4, when the temperature was increased quickly with large power.

#### Example 3

Using the PTC heater of the seamless cylinder shape and the flexible type to be set in close fit to the inside surface of

the photosensitive member, as illustrated in FIGS. 8A and 8B, without use of the temperature control circuit, several types of photosensitive members having different thicknesses of the conductive substrate and different outside diameters of the cylinder were prepared and set in the test machine. Then the heater was activated with the optimum power according to the heat capacity of the photosensitive member, the temperature of the photosensitive member was controlled to 45°C., and time changes of temperature were measured during a continuous sheet pass operation under an ambient at 15°C. The results are shown in FIG. 11 and the measurement results are shown in Table 5.

TABLE 5

| Dynamic test (PTC) | Outside diameter |    |    |    |    |     |
|--------------------|------------------|----|----|----|----|-----|
|                    | 10               | 20 | 30 | 60 | 80 | 108 |
| Thickness          | 0.05             | —  | —  | —  | —  | —   |
|                    | 0.10             | —  | Δ  | Δ  | ○  | ○   |
|                    | 0.50             | —  | Δ  | ○  | ○  | ○   |
|                    | 1.00             | —  | ○  | ○  | ○  | ○   |
|                    | 1.50             | —  | ○  | ○  | ○  | ○   |
|                    | 2.00             | —  | ○  | ○  | ○  | ○   |
|                    | 2.50             | —  | ○  | ○  | ○  | ○   |
|                    | 3.00             | —  | ○  | ○  | ○  | ○   |
|                    | 3.50             | —  | ○  | ○  | ○  | ○   |
|                    | 5.00             | —  | ○  | ○  | ○  | ○   |

Criteria for evaluation:

- very good,
- good,
- Δ practically acceptable,
- unmeasurable

Criteria for evaluation: ○ very good, ○ good, Δ practically acceptable, —unmeasurable

The photosensitive drums of the substrate 0.05 mm thick suffered film peeling off during the deposition or during the measurement because of their insufficient strength and the measurement was impossible therewith.

FIG. 11 shows a typical example of the actual measurement and, as shown in Table 5, the good results were obtained for all the samples with little dependence on the outside diameter by using the optimum power according to the heat capacity of the photosensitive member. The results were better, particularly, with the thick samples, because they had a large heat capacity.

When this structure was employed, there appeared no time changes of temperature (or temperature control ripples) even in the dynamic state and no potential unevenness due to the aforementioned temperature characteristics, and the fine image density irregularities, which appeared before during the continuous sheet pass operation, were overcome.

Since the structure was free of the potential unevenness, potential control variations or controlled potential changes due to the potential unevenness caused by temperature characteristics, encountered before, were eliminated in the so-called "potential control" to control latent image conditions by charge quantity, light quantity, etc. with provision of potential measuring means, so as to improve convergence of potential, thereby enhancing stability of image density further.

#### Comparative Example 2

Using the temperature control circuit as illustrated in FIG. 6 and using a heater of the seamless cylinder shape and the flexible type to be set in close fit to the inside surface of the photosensitive member, several types of photosensitive members having different thicknesses of the conductive substrate and different outside diameters of the cylinder

were prepared and set in the test machine. Then the heater was activated with the power of Example 3 according to the heat capacity of the photosensitive member, the temperature of the photosensitive member was controlled to 45°C., and time changes of temperature were measured during the continuous sheet pass operation under an ambient at 15°C. FIG. 12 shows an example of the results of the measurement. The measurement results are shown in Table 6.

TABLE 6

| Thickness | Dynamic test (conventional) | Outside diameter |    |    |    |    |     |
|-----------|-----------------------------|------------------|----|----|----|----|-----|
|           |                             | 10               | 20 | 30 | 60 | 80 | 108 |
| 0.05      | —                           | —                | —  | —  | —  | —  | —   |
| 0.10      | —                           | Δ                | Δ  | ○  | ○  | ○  | ○   |
| 0.50      | —                           | Δ                | ○  | ○  | ○  | ○  | ○   |
| 1.00      | —                           | ○                | ○  | ○  | ○  | ○  | ○   |
| 1.50      | —                           | ○                | ○  | ○  | ○  | ○  | ○   |
| 2.00      | —                           | ○                | ○  | ○  | ○  | ○  | ○   |
| 2.50      | —                           | ○                | ○  | ○  | ○  | ○  | ○   |
| 3.00      | —                           | ○                | ○  | ○  | ○  | ○  | ○   |
| 3.50      | —                           | ○                | ○  | ○  | ○  | ○  | ○   |
| 5.00      | —                           | ○                | ○  | ○  | ○  | ○  | ○   |

Criteria for evaluation:

- good,
- Δ practically acceptable,
- possibly problematic in practical use,
- unmeasurable

Criteria for evaluation: ○ good, Δ practically acceptable, —possibly problematic in practical use, —unmeasurable

The photosensitive drums of the substrate 0.05 mm thick suffered film peeling off during the deposition or during the measurement because of their insufficient strength and the measurement was impossible therewith.

As illustrated in FIG. 12, because the large power was supplied in order to compensate for the temperature decrease due to the sheet pass, there appeared the temperature control ripples and there also appeared the potential unevenness and image density irregularities due to the aforementioned temperature characteristics.

#### Example 4

Using the deposited film forming system by the VHF-PCVD method illustrated in FIG. 4, the electrophotographic, photosensitive members of the inhibition type were produced under the conditions of Table 7 according to the aforementioned procedures of the deposited film forming method. The thickness of the photoconductive layer was 20  $\mu\text{m}$ . In the present example, six aluminum supports were prepared in the outside diameter of 80 mm and in the thickness range of 0.1 mm to 2.5 mm, as shown in Table 8. The supports, after cut, were cleaned with pure water and a surface active agent and thereafter rinsed well with pure water. Then they were dried.

TABLE 7

|                | Inhibiting layer                                                                                                   | Photoconductive layer                                    | Surface protecting layer                                 |
|----------------|--------------------------------------------------------------------------------------------------------------------|----------------------------------------------------------|----------------------------------------------------------|
| Gas species    | SiH <sub>4</sub> : 300 sccm<br>H <sub>2</sub> : 500 sccm<br>NO: 8 sccm<br>B <sub>2</sub> H <sub>6</sub> : 2000 ppm | SiH <sub>4</sub> : 500 sccm<br>H <sub>2</sub> : 500 sccm | SiH <sub>4</sub> : 50 sccm<br>CH <sub>4</sub> : 500 sccm |
| Power          | 100 W                                                                                                              | 400 W                                                    | 300 W                                                    |
| Inner pressure | 0.018 Torr                                                                                                         | 0.020 Torr                                               | 0.020 Torr                                               |
| Thickness      | 3.0 $\mu\text{m}$                                                                                                  | 20.0 $\mu\text{m}$                                       | 0.5 $\mu\text{m}$                                        |

TABLE 8

| Support        | A1  | B1  | C1  | D1  | E1  | F1  |
|----------------|-----|-----|-----|-----|-----|-----|
| Thickness [mm] | 0.1 | 0.5 | 1.0 | 1.5 | 2.0 | 2.5 |

Each of the photosensitive drums for electrophotography obtained in this way was mounted in the electrophotographic apparatus for tests modified for the tests from NP6750 (trade name) manufactured by CANON K.K. and images were formed thereby. Then the influence of film peeling off was evaluated. The results are shown in Table 9.

Table 10 shows the results of the measurement of roundness of the photosensitive members for electrophotography produced. Numerical values in Table 10 are differences between the most depressed part and the most projecting part.

TABLE 9

| Thickness [mm]                       | 0.1 | 0.5 | 1.0 | 1.5 | 2.0 | 2.5 |
|--------------------------------------|-----|-----|-----|-----|-----|-----|
| Number of film peeled off portions A | 8   | 6   | 4   | 3   | 1   | 0   |
| Number of film peeled off portions B | 2   | 1   | 0   | 0   | 0   | 0   |
| Evaluation of image                  | Δ   | Δ   | ○   | ○   | ◎   | ◎   |

Criteria for image evaluation:

◎ very good,

○ good,

Δ practically acceptable

A: sizes of film peeled off portions  $0.3 \text{ mm} \leq \Phi \leq 0.6 \text{ mm}$

B: sizes of film peeled off portions  $0.6 \text{ mm} < \Phi$

Criteria for image evaluation: ◎ very good, ○ good, Δ practically acceptable

A: sizes of film peeled off portions  $0.3 \text{ mm} \leq \Phi \leq 0.6 \text{ mm}$

B: sizes of film peeled off portions  $0.6 \text{ mm} < \Phi$

TABLE 10

| Thickness [mm]                          | 0.1 | 0.5 | 1.0 | 1.5 | 2.0 | 2.5 |
|-----------------------------------------|-----|-----|-----|-----|-----|-----|
| Degree of deformation [ $\mu\text{m}$ ] | 60  | 35  | 40  | 30  | 10  | 15  |

As seen from Table 9 and Table 10, the film peeling off and the deformation of the support after the deposition were able to be suppressed to the minimum with the photosensitive members for electrophotography prepared by the plasma CVD method to induce the discharge at the discharge frequency not less than 50 MHz nor more than 450 MHz, because the stress of the deposited film was small even in the thickness of the support of not less than 0.1 mm but less than 2.5 mm.

### Comparative Example 3

Using the deposited film forming system by the RF-PCVD method illustrated in FIG. 4, the electrophotographic, photosensitive members of the inhibition type were produced under the conditions of Table 11 according to the aforementioned procedures of the deposited film forming method. The thickness of the photoconductive layer was 20  $\mu\text{m}$ . In the present example, six aluminum supports were prepared in the outside diameter of 80 mm and in the thickness range of 0.1 mm to 5.0 mm, as shown in Table 12. The supports, after cut, were cleaned with pure water and the surface active agent and thereafter rinsed well with pure water. Then they were dried.

TABLE 11

|                | Inhibiting layer                                                                                                   | Photoconductive layer                                    | Surface protecting layer                                 |
|----------------|--------------------------------------------------------------------------------------------------------------------|----------------------------------------------------------|----------------------------------------------------------|
| Gas species    | SiH <sub>4</sub> : 300 sccm<br>H <sub>2</sub> : 500 sccm<br>NO: 8 sccm<br>B <sub>2</sub> H <sub>6</sub> : 2000 ppm | SiH <sub>4</sub> : 500 sccm<br>H <sub>2</sub> : 500 sccm | SiH <sub>4</sub> : 50 sccm<br>CH <sub>4</sub> : 500 sccm |
| Power          | 100 W                                                                                                              | 400 W                                                    | 300 W                                                    |
| Inner pressure | 0.4 Torr                                                                                                           | 0.5 Torr                                                 | 0.5 Torr                                                 |
| Thickness      | 3.0 $\mu\text{m}$                                                                                                  | 20.0 $\mu\text{m}$                                       | 0.5 $\mu\text{m}$                                        |

TABLE 12

| Support        | A2  | B2  | C2  | D2  | E2  | F2  |
|----------------|-----|-----|-----|-----|-----|-----|
| Thickness [mm] | 0.1 | 0.5 | 1.5 | 2.5 | 3.0 | 5.0 |

Each of the photosensitive drums for electrophotography obtained in this way was mounted in the electrophotographic apparatus for tests modified for the tests from NP6750 (trade name) of CANON K.K. and images were formed thereby. Then the influence of film peeling off was evaluated. The results are shown in Table 13.

Table 14 shows the results of the measurement of roundness of the photosensitive members for electrophotography produced. Numerical values in Table 14 are differences between the most depressed part and the most projecting part.

TABLE 13

| Thickness [mm]                       | 0.1 | 0.5 | 1.5 | 2.5 | 3.0 | 5.0 |
|--------------------------------------|-----|-----|-----|-----|-----|-----|
| Number of film peeled off portions A | 50  | 25  | 22  | 5   | 1   | 1   |
| Number of film peeled off portions B | 20  | 7   | 7   | 1   | 0   | 0   |
| Evaluation of image                  | x   | x   | x   | Δ   | ○   | ◎   |

Criteria for image evaluation:

◎ very good,

○ good,

Δ practically acceptable,

x possibly problematic in practical use

A: sizes of film peeled off portions  $0.3 \text{ mm} \leq \Phi \leq 0.6 \text{ mm}$

B: sizes of film peeled off portions  $0.6 \text{ mm} < \Phi$

Criteria for image evaluation: ◎ very good, ○ good, Δ practically acceptable, x possibly problematic in practical use

A: sizes of film peeled off portions  $0.3 \text{ mm} \leq \Phi \leq 0.6 \text{ mm}$   
B: sizes of film peeled off portions  $0.6 \text{ mm} < \Phi$

TABLE 14

| Thickness [mm]                           | 0.1 | 0.5 | 1.5 | 2.5 | 3.0 | 5.0 |
|------------------------------------------|-----|-----|-----|-----|-----|-----|
| Degree of deformation [ $\mu\text{m}$ ]* | 150 | 230 | 100 | 80  | 10  | 20  |

\*A problem could be posed if the degree of deformation is over 60  $\mu\text{m}$ .

\*A problem could be posed if the degree of deformation is over 60  $\mu\text{m}$ .

As seen from Table 13 and Table 14, the photosensitive members for electrophotography prepared by the plasma CVD method to induce the discharge at the discharge frequency (13.56 MHz) in the RF band and having the support of the outside diameter of 80 mm suffered the film peeling off/the deformation of the support after the deposition because of the stress in the deposited film unless the thickness of the support was not less than 2.5 mm.

## Example 5

Each of the photosensitive members for electrophotography prepared in Example 4 was mounted on the electrophotographic apparatus modified from NP6750 (trade name) of CANON K.K. and was subjected to evaluation of image and evaluation as to surface deviation during the mounted state on the electrophotographic apparatus. The image evaluation was conducted by checking a level of image nonuniformity due to the surface deviation, and image defects. The heater illustrated in FIG. 5A and FIG. 5B and the temperature control circuit were set inside the photosensitive member and controlled so that the temperature of the photosensitive member became 45° C. The results are shown in Table 15.

TABLE 15

| Thickness [mm]               | 0.1 | 0.5 | 1.0 | 1.5 | 2.0 | 2.5 |
|------------------------------|-----|-----|-----|-----|-----|-----|
| Image defects                | Δ   | Δ   | ○   | ○   | ○   | ◎   |
| Image blur                   | Δ   | ○   | ○   | ○   | ○   | ◎   |
| Image density irregularities | Δ   | Δ   | ○   | ○   | ○   | ◎   |

Criteria for image evaluation:

◎ very good,

○ good,

Δ practically acceptable

Criteria for image evaluation: ◎ very good, ○ good, Δ practically acceptable

As shown in Table 15, the very good results were obtained in the electrophotographic apparatus incorporating the photosensitive member of the present invention. Namely, it was made possible to obtain the good electrophotographic apparatus with suppressing the film peeling off/the deformation of the support to the minimum even in the thickness of the support not less than 0.1 mm but less than 2.5 mm because of the small stress in film if a-Si was laid by the VHF-PCVD method at the frequency not less than 50 MHz nor more than 450 MHz.

When the drum-like metal substrate used was the one having the thickness not less than 0.1 mm but less than 2.5 mm and when the heater was used for the control of temperature of the photosensitive member, the temperature was able to be controlled with high accuracy, because the temperature gradient was small between the heater and the surface of the photosensitive member, and very good images were able to be obtained with stable density even in the continuous sheet pass operation.

## Example 6

Using the PTC heater of the seamless cylinder shape and the flexible type to be set in close fit to the inside surface of the photosensitive member, as illustrated in FIG. 8B, without use of the temperature control circuit, each of the photosensitive members for electrophotography prepared in Example 4 was set in a test machine modified from NP6750 (trade name) of CANON K.K. Then the heater was activated with the optimum power according to the heat capacity of the photosensitive member and time changes of temperature were measured in the static state in which the temperature of the photosensitive member was controlled to 45° C., after the start of power supply to the heater. The results were time changes as illustrated in FIG. 9, similar to those in Example 2.

A typical example of the actual measurement was the tendency as illustrated in FIG. 9. Almost the same tendency was observed at all measured portions on the photosensitive member. When the temperature was increased quickly with large power, there appeared no temperature difference

depending upon locations upon switching nor time changes of temperature (temperature control ripples) at the measured portions. Further, the good results were obtained for all the samples with little dependence on the thickness of the support by using the optimum power according to the heat capacity of the photosensitive member. The results were better, particularly, with the samples of the support having the thickness less than 2.5 mm.

## Comparative Example 4

Using the temperature control circuit as illustrated in FIG. 6 and also using the heater of the type with the seam in which the flat sheet heater was curved so as to closely fit the inside surface of the photosensitive member, and the heater of the seamless cylinder shape and of the flexible type to closely fit the inside surface of the photosensitive member, each of the photosensitive members for electrophotography prepared in Example 4 was set in the test machine modified from NP6750 (trade name) manufactured by CANON K.K. Then the heater was activated with the power of Example 6 according to the heat capacity of the photosensitive member and time changes of temperature were measured in the static state in which the temperature of the photosensitive member was controlled to 45° C., after the start of power supply to the heater. The results of the time changes of temperature demonstrated the tendencies as shown in FIG. 10, similar to those in Comparative Example 1.

In FIG. 10, in the case of the heater of the type with the seam, the temperature changes were as indicated by the solid line at a portion which was not the seam of the heater and as indicated by the dashed line at the seam portion of the heater. There was thus a large temperature difference between them upon switching. On the other hand, in the case of the heater of the type without the seam, the temperature changes were as indicated by the solid line at all the measured portions, and there was no temperature difference depending upon locations upon switching. However, there appeared time changes of temperature (temperature control ripples) at the measured portions.

Even with the heaters of these types which posed no practical problem under the conventional, practical use conditions, the tendencies as described above became more prominent, particularly, with the thick samples when the temperature was increased quickly with large power.

## Example 7

Using the PTC heater of the seamless cylinder shape and the flexible type to be set in close fit to the inside surface of the photosensitive member, as illustrated in FIG. 8B, without use of the temperature control circuit, each of the photosensitive members for electrophotography prepared in Example 4 were set in the test machine modified from NP6750 (trade name) of CANON K.K. Then the heater was activated with the optimum power according to the heat capacity of the photosensitive member and controlled so that the temperature of the photosensitive member became 45° C., and time changes of temperature was measured in the continuous sheet pass operation under the ambient at 15° C. The results demonstrated the tendency as shown in FIG. 11, similar to that in Example 3.

The photosensitive drums of the support 0.05 mm thick suffered film peeling off during the deposition or during the measurement because of their insufficient strength and the measurement was impossible therewith.

As shown in FIG. 11, the good results were obtained for all the samples by using the optimum power according to the

heat capacity of the photosensitive member. The results were better, particularly, with the thick samples, because they have a large heat capacity.

When this structure was employed, there appeared no time changes of temperature (temperature control ripples) even in the dynamic state and no potential unevenness due to the aforementioned temperature characteristics, and the fine image density irregularities, which appeared before during the continuous sheet pass operation, were overcome.

Since the structure was free of the potential unevenness, potential control variations or controlled potential changes due to the potential unevenness caused by temperature characteristics, encountered before, were eliminated in the so-called "potential control" to control latent image conditions by charge quantity, light quantity, etc. with provision of potential measuring means, so as to improve convergence of potential, thereby enhancing the stability of image density further.

#### Comparative Example 5

Using the temperature control circuit as shown in FIG. 6 and using the heater of the seamless cylinder shape and the flexible type to closely fit the inside surface of the photosensitive member, each of the photosensitive members for electrophotography prepared in Example 4 was set in the test machine modified from NP6750 (trade name) of CANON K.K. and the heater was energized by supplying the power of Example 6 according to the heat capacity of the photosensitive member and controlled so that the temperature of the photosensitive member became 45° C. The time changes of temperature were measured in the continuous sheet pass operation under the ambient at 15° C. The results were as shown in FIG. 12, similar to those in Comparative Example 2.

In this comparative example, as shown in FIG. 12, because the large power was supplied in order to compensate for the temperature decrease due to the sheet pass, there appeared the temperature control ripples and there also appeared the potential unevenness and image density irregularities due to the aforementioned temperature characteristics.

As detailed above, the present invention can provide the electrophotographic, photosensitive member and the image forming apparatus capable of stably providing high-quality images and permitting cost reduction toward improvement in the temperature characteristics.

In addition, the present invention can provide the electrophotographic, photosensitive member permitting the power savings in the production of the electrophotographic, photosensitive member, the decrease of tact time, and the reduction of the production cost, and the image forming apparatus having the photosensitive member.

Further, the present invention can provide the electrophotographic, photosensitive member that can present high-quality images with fewer image defects such as blank area or the like due to the film peeling off of the a-Si(H,X) deposited film and that can be produced at low cost, and the electrophotographic apparatus having the electrophotographic, photosensitive member.

In addition, the present invention can provide the electrophotographic apparatus using the photoconductive member for electrophotography with excellent durability, which can always demonstrate the stable, electrical, optical, and photoconductive characteristics and which suffers no deterioration even in repetitive use.

The electrophotographic, photosensitive member of a-Si(H,X) according to the present invention is formed by the

plasma CVD method to induce the discharge at the discharge frequency not less than 50 MHz nor more than 450 MHz, whereby the stress in the film can be made very small. Namely, it becomes possible to use the conductor support not less than 0.1 mm but less than 2.5 mm, which contributes very much to the cost reduction, based on the power savings and the decrease of the tact time because of the decrease of the heating time in the production of the a-Si(H,X) film, the cutback of the high-temperature-maintaining power, the decrease of the tact time because of the decrease of the cooling time, and so on.

Further, according to the present invention, the drum-like metal substrate used is the one having the outside diameter not less than 20 mm nor more than 60 mm, whereby the degree of thermal deformation of the drum-like metal substrate can be suppressed to the sufficiently small level even if the drum-like metal substrate is heated during the production of the photoconductive member and during the use as a photosensitive drum for electrophotography; therefore, the level of the film peeling off of the a-Si(H,X) deposited film can be controlled to the level in which no problem is posed in the practical use, or to zero, and the thickness of the drum-like metal substrate can be not less than 0.1 mm but less than 2.5 mm, thereby permitting the production cost to be curtailed drastically.

When the heater is used in the drum-like metal substrate having the thickness of not less than 0.1 mm but less than 2.5 mm, the high-accuracy temperature control can be effected, because the temperature gradient is small between the heater and the surface of the photosensitive member.

Further, the use of the PTC heater in the seamless structure permits the input of much higher power than for the temperature equilibrium state, so as to increase the response; therefore, quick temperature increase can be performed on one hand and the temperature control can be effected without the overshoots nor temperature control ripples even in the dynamic state with the sheet pass operation on the other hand.

What is claimed is:

1. An electrophotographic, photosensitive member which is cylindrical and comprises a photosensitive layer comprising amorphous silicon provided on an electroconductive substrate, and in which the thickness of the electroconductive substrate is not less than 0.1 mm but less than 2.5 mm, wherein the photosensitive layer is a layer formed by a plasma CVD method to induce a discharge at a discharge frequency of not less than 50 MHz nor more than 450 MHz.

2. An electrophotographic apparatus comprising the electrophotographic, photosensitive member as set forth in claim 1.

3. The electrophotographic apparatus according to claim 2, wherein the electrophotographic, photosensitive member has the electroconductive substrate of a drum shape, and wherein a heater is provided inside a hollow part of the substrate, the heater being a heat-generating member having a positive temperature coefficient of resistance.

4. The electrophotographic, photosensitive member according to claim 1, wherein the base material of the electroconductive substrate is aluminum or an aluminum base alloy.

5. The electrophotographic apparatus according to claim 3, wherein the base material of the electroconductive substrate is aluminum or an aluminum base alloy.

6. The electrophotographic apparatus comprising:

(a) an electrophotographic photosensitive member comprising a photosensitive layer comprising amorphous silicon on a cylindrical electroconductive substrate; and

**29**

(b) a heat-generating member having a positive temperature coefficient of resistance spaced inside electrophotographic photosensitive member, wherein the cylindrical electroconductive substrate has a thickness in the range from 0.1 mm to less than 2.5 mm and an outside diameter from 20 mm to 60 mm.

7. The electrophotographic apparatus according to claim 6, wherein an exterior surface of the heat generating member

5 congruently contacts a corresponding interior surface of the photosensitive member.

8. The electrophotographic apparatus according to claim 6, wherein the base material of the electroconductive substrate is aluminum or an aluminum base alloy.

\* \* \* \* \*

UNITED STATES PATENT AND TRADEMARK OFFICE  
**CERTIFICATE OF CORRECTION**

PATENT NO. : 6,110,629  
DATED : August 29, 2000  
INVENTOR(S) : Toshiyuki Ehara et al.

Page 1 of 2

It is certified that error appears in the above-identified patent and that said Letters Patent is hereby corrected as shown below:

Title page,

Item [56] References Cited, under U.S. PATENT DOCUMENTS  
“Shiral” should read -- Shirai --; and “Nakumura” should read -- Nakamura --;

Under FOREIGN PATENT DOCUMENTS

Insert: -- 0594453 4/94 Europe --;  
-- 2018446 10/79 Great Britain --;  
-- 2102028 1/83 Great Britain --;  
-- 0136902 14/85 Europe --;  
--0168148 1/86 Europe --;

Under OTHER PUBLICATIONS

Insert: -- Patent Abstracts of Japan, Vol. 98, No. 2, 1/28 For JP-9-283448. --;  
-- Database WPI Sec. CH, Wk 8822, Derwent Publ., AN88 — 151079  
(1988) . --;  
--Database WPI Sec. CH, Wk 8827, Derwent Publ., AN88 — 185758 (1988). --.

Column 4,

Line 20, “yet” (second occurrence) should be deleted.

Column 5,

Line 3, “tact” should read -- tack --.

Column 21,

Line 49, “before” should read -- before and --.

Column 24,

Line 65, “off/the” should read -- off the --.

Column 27,

Line 7, “before” should read -- before and --;

Line 55, “of” should be deleted.

Column 28,

Line 19, “of” should be deleted.

UNITED STATES PATENT AND TRADEMARK OFFICE  
**CERTIFICATE OF CORRECTION**

PATENT NO. : 6,110,629  
DATED : August 29, 2000  
INVENTOR(S) : Toshiyuki Ehara et al.

Page 2 of 2

It is certified that error appears in the above-identified patent and that said Letters Patent is hereby corrected as shown below:

Column 29,  
Line 2, "inside" should read -- inside the --.

Signed and Sealed this

Twenty-third Day of October, 2001

Attest:

*Nicholas P. Godici*

Attesting Officer

NICHOLAS P. GODICI  
Acting Director of the United States Patent and Trademark Office